# EUROPEAN PATENT SPECIFICATION

(11) **EP 0 235 130 B1**
(45) Date of publication and mention of the grant of the patent: **03.01.1990**
(21) Application number: 85905539.4
(22) Date of filing: 25.10.1985
(51) Int. Cl.: D06N 7/00, B32B 29/02

(54) **FLAME-PROOF COVERING INTENDED FOR WALLS AND OTHER SURFACES AND A METHOD FOR THE MANUFACTURE OF THE SAME**
FLAMMSCHUTZDECKMATERIAL FÜR WÄNDE ODER SONSTIGE OBERFLÄCHEN UND DESSEN HERSTELLUNGSVERFAHREN
REVETEMENT ININFLAMMABLE POUR MURS ET AUTRES SURFACES ET METHODE DE FABRICATION DUDIT REVETEMENT

(30) Priority: 01.11.1984 SE 8405463
(43) Date of publication of application: 09.09.1987
(73) Proprietor: FRANSSON, Bill, S-430 20 Veddige (SE)
(72) Inventor: FRANSSON, Bill, S-430 20 Veddige (SE)
(74) Representative: Grams, Klaus Dieter, Dipl.-Ing.
(86) International application number: SE8500415
(87) International publication number: WO8602675

(56) References cited:
- EP-A- 0 016 456
- FR-A- 2 217 158
- GB-A- 2 024 711

## Description

The present invention relates to a flame-proof covering intended for walls and other surfaces according to the preamble of claim 1, and to a method for manufacture thereof, according to the preamble of claim 3. A covering of this kind is known from EP-A-0 016 456.

In previous attempts to produce flame-proof wall surfaces, etc., through the use of wall coverings for said purpose, these were found to be costly to manufacture and difficult to handle when putting up, and required lengthy treatment in conjunction with their preparation, since it was necessary, amongst other things, to wait for a full day before painting over them. These are some of the reasons why glass fibre materials have accounted for a very small proportion of the products available on the ordinary consumer market. Glass fibre products are instead used to an overwhelming extent in the public sector, where there has been good access to skilled staff. The principal object of the present invention is thus primarily to attempt to solve said problems.

Said object is achieved by means of a covering as specified above and further defined in the characterising portion of Claim 1.

The invention also relates to a method for manufacturing a covering of said kind in an efficient and simple fashion. This method, already specified above, is further defined in the characterising portion of Claim 3.

The invention is described below in the form of a preferred illustrative embodiment, in conjunction with which reference is made to the following drawings, of which:
Fig. 1 is a diagrammatic representation of different stages in the manufacture of a covering according to the invention;
Fig. 2 shows a transverse section through a manufactured covering;
Fig. 2A shows on an enlarged scale a part of the covering; and
Fig. 3 shows a typical pattern of a manufactured covering.

From bobbins 1, for example, or other storage rollers which have wound onto them glass yarn 2 made from glass fibre material, the fibre yarn threads 2 in question are fed in such a way that, once they have been deflected, if necessary, around deflectors 3 in the direction of the arrows 4, from a first station I, they can be routed in parallel in relation to one another in the direction of feed by being deflected around further deflector devices 5 at a second station 11.

The threads 2 are then fed in the direction of the arrow 6, after having been compressed between rollers 7,8, for example, to a third station III. The operations performed at this station III include the attachment of threads 2 to a carrier 10 for the proposed covering 9 according to the invention executed as wallpaper. Said carrier 10 is made of paper, and may exhibit the form of an extended strip which is wound so as to form a roll 11, from which it can be fed in the direction of the arrow 12 to a consolidating device 13. Before arriving at, or on passing through the device 13, the carrier 10 is intended to receive a coating of a securing layer 14, consisting of a bonding agent, which exhibits the ability to be flame-proof and which may also be pigmented as appropriate with the desired colour. For example, a container 15 may, for the purpose of forming said securing layers in a dried and/or cured state, contain the intended substance 16 in a non-hardened state, and which may be applied, for example, to the carrying strip 10 preferably along the entire length of one of its side surfaces 10A, by means of a roller 17, which runs in said container 15 and substance 16. As it is deflected around a roller 18, etc., in the arrangement 13 for the strip 10 and the threads 2, the threads 2 are applied to the base layer 14 of the adhesive coated along the strip 10. As it subsequently passes through a nip between, for example, said roller 18 and a press roller 19 operating in conjunction with same in the direction of the arrow 20, the threads 2 are compressed in such a way that they are pressed with their sides 2A facing the carrier 10 down into the as yet unhardened or uncured base layer 14, which is intended, in addition to serving for attachment purposes and as a flame guard for the manufactured wallpaper 9, also to produce a background colour effect in the wallpaper 9, depending on whether the layer 14 is pigmented with the intended colour.

The strip 10 is then allowed to dry/cure with the threads applied to it, said threads running parallel in relation to one another and essentially in the same direction as the longitudinal sense of the strip. Drying/curing may take place at a subsequent fourth station IV, which may exhibit an appropriate number of winding rollers 21, 22, etc., around which the manufactured wallpaper 9 is wound, for example in a heating oven.

At a fifth and subsequent station V, a flame-proof surface coating 23, preferably also pigmented in the desired colour, is applied along that side 2B of the threads 2 attached to the carrier 10 which face in a direction away from the carrier 10. Said outer layer 23 may be applied to the threads 2 by the use of a scraping action on the layer 23, such that only the outer sides 2B or the raised parts of the threads which project up out of the base layer 14 are coated with said outer layers 23, whereby a coloured effect of the threads 2 is achieved against the background of any underlying colour of the base layer 14. Another method for the application of the outer layer 23 is also permissible, for example by the user of a roller, etc.

Said outer layer is then also allowed by dry in a suitable fashion, whereupon the strip of wallpaper 9, which is moving in the direction of the arrow 24, is conveyed for subsequent general wallpaper processing operations, such as rolling and cutting, etc.

The covering manufactured in the form of a wallpaper 9, which is suitable for attachment to walls and other surfaces of an appropriate kind, can be hung on a wall, for example, in the customary fashion, as in the case of conventional wallpapers, thus enabling a flame-proof covering of the desired colour to be provided by the simple and rapid installation of the desired wallpaper 9, which can even be done by persons without full training.

The invention is not restricted to the illustrative embodiment described above and shown in the drawings. For example, threads may be juxtaposed with strips of glass fibre material.

## Claims

1. Flame-proof covering for walls and other surfaces in the form of a wallpaper (9) which exhibits a carrier (10) made of paper and comprising a flame-proof base bonding layer (14) coated on the carrier, characterized by glass fibre threads (2) formed by bundles of threads made of glass yarn pushed down (side 2A) into the flame-proof base layer (14), but having raised parts which project up out of the layer (14), and extending essentially parallel to each other and essentially in the same direction as the longitudinal direction of the wallpaper at a certain distance from one another, measured in the transverse direction of the threads; and by a flame-proof and pigmented outer layer (23) applied on the outer sides (2B) of the raised parts of the threads (2) which face away from the carrier (10).

2. Flame-proof covering according to Patent Claim 1, characterized in that the base layer (14) is pigmented in such a way as to achieve a coloured background effect on the wallpaper (9).

3. Method for the manufacture of a flame-proof covering according to Claim 1 or 2, characterized in that a number of glass fibre threads (2), which are formed by bundles of threads made of glass yarn, are routed in parallel to each other and attached to a parallely running carrier (10) by pushing them down (side 2A) into a flame-proof base layer (14) of a bonding agent previously coated on the carrier, in a way that the threads (2) have raised parts which project up out of the layer (14) and extend essentially parallel to each other and essentially in the same direction as the longitudinal direction of the wallpaper at a certain distance from one another, measured in the transverse direction of the threads; and in that externally along the threads (2) on that side (2B) of the same which faces away from the carrier (10), a flame-proof and pigmented outer layer (23) is applied in such a way that only outer threads (2B) or the raised parts of the threads (2) are coated with said outer layer (23).

4. Method according to Claim 3, characterized in that the said flame-proof base layer (14) of a bonding agent is pigmented, in such a way as to achieve a coloured background effect on the wallpaper (9).

5. Method according to one of the Claims 3 or 4, characterized in that the glass fibre threads (2) are unwound from rolls (1) and pushed down into the base layer of bonding agent (14) between two rolls (18,19).

6. Method according to one of the Claims 3 to 5, characterized in that the flame-proof, pigmented outer layer (23) is applied to the threads (2) after drying the bonding layer (14) applied to the carrier (10).

7. Method according to Claim 6, characterized in that said pigmented outer layer (23) is applied to the threads (2) by means of a scraping action.

## Patentansprüche

1. Flammschutzüberzug für Wände oder sonstige Oberflächen in Form einer Tapete (9), die einen Träger (10) umfaßt, der aus Papier besteht, und eine Flammschutz-Basisbindeschicht (14) aufweist, die auf den Träger aufgebracht ist, gekennzeichnet durch Glasfaserfäden (2), die von Bündeln von aus Glasgarn bestehenden Fäden gebildet sind, nach unten (Seite 2A) in die Flammschutz-Basisschicht (14) gedrückt sind, aber erhöhte Abschnitte haben, die nach oben aus der Schicht (14) hervorstehen, und im wesentlichen parallel zueinander sowie im wesentlichen in der gleichen Richtung wie die Längsrichtung der Tapete in einem in Querrichtung der Fäden gemessenen, gewissen Abstand voneinander verlaufen, und durch eine flammschützende und pigmentierte äußere Schicht (23), die auf den Außenseiten (2B) der erhöhten Abschnitte der Fäden (2), die von dem Träger (10) abgewandt sind, angebracht ist.

2. Flammschutzüberzug nach Anspruch 1, dadurch gekennzeichnet, daß die Basisschicht (14) derart pigmentiert ist, daß ein farbiger Hintergrundeffekt auf der Tapete (9) erzielt wird.

3. Verfahren zur Herstellung eines Flammschutz- überzuges nach Anspruch 1 oder 2, dadurch gekennzeichnet, daß eine Anzahl von Glasfaserfäden (2), die von einem Bündel von aus Glasgarn bestehenden Fäden gebildet sind, parallel zueinander geführt und an einem parallel verlaufenden Träger (10) angebracht werden, indem sie nach unten (Seite 2A) in eine Flammschutz-Basisschicht (14) eines vorher auf dem Träger angebrachten Bindemittels derart gedrückt werden, daß die Fäden (2) erhöhteAbschnitte haben, die nach oben aus der Schicht (14) hervorstehen, und im wesentlichen parallel zueinander sowie im wesentlichen in der gleichen Richtung wie die Längsrichtung der Tapete in einem in Querrichtung der Fäden gemessenen, gewissen Abstand voneinander verlaufen, und daß außen entlang der Fäden (2) auf deren Seite (2B), die von dem Träger (10) abgewandt ist, eine flammschützende und pigmentierte äußere Schicht (23) derart aufgebracht wird, daß nur äußere Fäden (2B) oder die erhöhten Abschnitte der Fäden (2) mit der äußeren Schicht (23) überzogen sind.

4. Verfahren nach Anspruch 3, dadurch gekennzeichnet, daß die Flammschutz-Basisschicht (14) eines Bindemittels derart pigmentiert ist, daß ein farbiger Hintergrundeffekt auf der Tapete (9) erzielt wird.

5. Verfahren nach Anspruch 3 oder 4, dadurch gekennzeichnet, daß die Glasfaserfäden (2) von Rollen (1) abgewickelt und zwischen zwei Walzen (18,19) in die Basisschicht (14) des Bindemittels hineingedrückt werden.

6. Verfahren nach einem der Ansprüche 3 bis 5, dadurch gekennzeichnet, daß die flammschützende, pigmentierte äußere Schicht (23) auf die Fäden (2) aufgebracht wird, nachdem die auf den Träger (10) aufgebrachte Bindeschicht (14) getrocknet ist.

7. Verfahren nach Anspruch 6, dadurch gekennzeichnet, daß die pigmentierte äußere Schicht (23) mittels eines Schabevorgangs auf die Fäden (2) aufgebracht wird.

## Revendications

1. Revêtement ignifuge pour murs ou autres surfaces, sous forme de papier peint (9) qui présente un support de papier (10) et comprend une couche de liant de base ignifuge (14), caractérisé par des fils en fibre de verre (2) formés par des faisceaux de fils obtenus à partir de fils de verre introduits à force (côté 2A) dans la couche de base ignifuge (14), mais ayant des portions qui dépassent de la couche (14) vers l'extérieur et s'étendent de façon pratiquement parallèle l'une à l'autre et sensiblement dans la même direction que la direction longitudinale du papier peint à une certaine distance l'une de l'autre mesurée transversalement à la direction des fils, et par une couche extérieure ignifuge pigmentée (23) appliquée sur les côtés extérieurs (2B) des parties dépassant des fils (2) qui font saillie du support (10).

2. Revêtement ignifuge selon la revendication 1, caractérisé en ce que la couche de base (14) est pigmentée de telle sorte qu'elle réalise un effet de coloration de fond du papier peint (9).

3. Procédé de fabrication d'un revêtement ignifuge selon la revendication 1 ou 2, caractérisé en ce que de nombreux fils de fibre de verre (2) qui sont formés en faisceaux de fils faits de fibres de verre sont dirigés parallèlement les uns aux autres et reliés à un support (10) se déroulant parallèlement par application de ceux-ci du côté (2A) dans une couche de base ignifuge (14) d'un liant préalablement déposé sur le support d'une façon telle que les fils (2) ont des portions qui dépassent de la couche (14) et s'étendent de façon pratiquement parallèle l'une à l'autre et pratiquement dans la même direction que le direction longitudinale du papier peint à une certaine distance l'une de l'autre, mesurée dans la direction transversale des fils; et en ce que extérieurement le long des fils (2) sur ce côté (2B) du même qui fait face en partant du support (10), on applique une couche extérieure ignifuge et pigmentée (23) d'une manière telle que seuls les fils extérieurs (2B), ou les portions relevées des fils (2) sont revêtus de cette couche extérieure (23).

4. Procédé selon la revendication 3, caractérisé en ce que la couche de base ignifuge (14) d'un liant est pigmentée de façon à réaliser un effet de fond coloré sur le papier peint (9).

5. Procédé selon l'une des revendications 3 ou 4, caractérisé en ce que les fils de fibre de verre (2) sont déroulés à partir de bobines (1) et enfoncés dans la couche de base du liant (14) entre deux rouleaux (18,19).

6. Procédé selon l'une des revendications 3 à 5, caractérisé en ce que la couche extérieure pigmentée ignifuge (23) est appliquée aux fils (2) après séchage du liant appliqué au support (10).

7. Procédé selon la revendication 6, caractérisé en ce que cette couche extérieure pigmentée (23) est appliquée aux fils (2) au moyen d'une action de grattage.
